

# United States Patent [19]

Ichinose et al.

[11] 3,899,451

[45] Aug. 12, 1975

[54] OXIDE VARISTOR

[75] Inventors: Noboru Ichinose; Yuhji Yokomizo,  
both of Tokyo, Japan

[73] Assignee: Tokyo Shibaura Electric Co., Ltd.,  
Kawasaki, Japan

[22] Filed: Sept. 11, 1973

[21] Appl. No.: 396,135

## [30] Foreign Application Priority Data

|                |            |          |
|----------------|------------|----------|
| Sept. 11, 1972 | Japan..... | 47-90446 |
| Sept. 11, 1972 | Japan..... | 47-90447 |
| Sept. 18, 1972 | Japan..... | 47-92897 |

[52] U.S. Cl..... 252/520; 252/518

[51] Int. Cl.<sup>2</sup>..... H01B 1/08

[58] Field of Search..... 252/520, 518

## [56] References Cited

### UNITED STATES PATENTS

3,669,907 6/1972 Kohashi et al..... 252/520 X

|           |         |                      |           |
|-----------|---------|----------------------|-----------|
| 3,778,743 | 12/1973 | Matsuoka et al. .... | 252/518 X |
| 3,805,114 | 4/1974  | Matsuoka et al. .... | 252/518 X |
| 3,806,765 | 4/1974  | Matsuoka et al. .... | 252/518 X |

Primary Examiner—Leland A. Sebastian  
Attorney, Agent, or Firm—Stewart and Kolasch, Ltd.

[57]

## ABSTRACT

An oxide varistor is prepared from a basic composition formed of 70 to 14 mol% of at least one  $Me^I_2O_2$ , 29 to 85 mol% of  $ZnO$  and 1 to 20 mol% of  $Sb_2O_3$ , 1 to 20% by weight of  $Bi_2O_3$ , and 0.5 to 10% by weight of at least one  $Me^{II}_2O_3$  based on said basic composition,  $Me^I$  being selected from Ti, Sn and Zr, and  $Me^{II}$  being selected from Fe, Cr, Mn and Co.

5 Claims, 14 Drawing Figures

FIG. 1



FIG. 2



FIG. 3A



FIG. 3B





FIG. 4A



FIG. 4B



FIG. 4C





FIG. 5B



FIG. 5C



FIG. 6A





FIG. 6C



## OXIDE VARISTOR

This invention relates to a varistor prepared from an oxide semiconductor, and more particularly to an oxide varistor having greater voltage-current nonlinear coefficient.

As one of circuit elements based on a semiconductor, a voltage nonlinear resistance element is known. SiC varistors are known as a typical example. The element of this kind has nonlinear voltage-current characteristics, namely, is sharply reduced in resistance with increasing voltage to permit electric current to be markedly increased accordingly and has consequently been widely used for absorbing abnormally high voltage or for stabilization of voltage.

With the recent marked advance in electronic art there is a growing demand for devices (IC, transistors, etc.) in which semiconductor are used. However, these electronic parts have disadvantage in common that they are weak against abnormal voltage and a settlement to this problem has been sought. Arresters, surge absorbers, etc., using the conventional SiC varistor are slow in charge response speed to impulses and incomplete for protection against surges involved in devices in which semiconductors are used.

With rotational devices, the art of breakers has been markedly developed. With the advent of a vacuum breaker, an on-off surge due to current suppression poses a problem. The protection against the on-off surge has heretofore been made by using a gap type arrester or a capacitor for electric power. In the gap type arrester, it is possible to absorb abnormal voltage due to a normal current suppression. However, there is still a problem in responding to impulses of the order of MHz in current unstable areas and impulses involved during re-ignition. When the capacitor is used, problems arise from the price consideration as well as from the setting of capacitance. Therefore, there is a demand for an inexpensive varistor element having excellent varistor characteristics.

Generally, the voltage-current characteristics of the varistor may be expressed approximately in the following equation:

$$I = (V/C)$$

where

I = current flowing through the varistor

V = voltage across the varistor

C = constant

$\alpha$  = nonlinear voltage coefficient

Therefore, the characteristics of the varistor may be indicated by C and  $\alpha$  or the two other constants which can replace them. Since accurate determination of C presents extreme difficulties, C is generally substituted by voltage  $V_c$  at a certain current C (mA). With the varistor voltage thus designated as  $V_c$  the voltage-current characteristics of the varistor may be indicated by  $V_c$  and the nonlinear coefficient  $\alpha$ . An SiC varistor heretofore well known as a varistor element has as small a voltage nonlinear coefficient  $\alpha$  as 3-7. A zener diode is known as having a larger voltage nonlinear coefficient. The zener diode is expensive and in addition has a limited usage voltage of 200 V at most and is consequently inconvenient for use with electronic devices requiring for high voltage. The zener diode involves a greater variation with temperature in the rising voltage

and a smaller surge resistance, thus presenting practical problems.

U.S. Pat. No. 3,632,529 discloses a voltage variable resistor ceramic composition consisting essentially of zinc oxide and 0.05 to 10.0 mol % of strontium oxide and, as an additive, 0.05 to 8.0 mol % of bismuth oxide, lead oxide, calcium oxide or cobalt oxide. This ceramic composition is different from an oxide semiconductor composition of an oxide varistor according to this invention. The voltage nonlinear coefficient of the ceramic composition is of the order of 10 and is lower than that (more than 30) of the oxide varistor according to this invention.

U.S. Pat. No. 3,663,458 discloses a nonlinear bulk-type resistor consisting essentially of a sintered body of 80.0 to 99.9 mol % of ZnO, 0.05 to 10 mol %  $\text{Bi}_2\text{O}_3$  and 0.05 to 10 mol % in total of at least one member selected from the group consisting of CoO, MnO<sub>2</sub>,  $\text{In}_2\text{O}_3$ ,  $\text{Sb}_2\text{O}_3$ ,  $\text{TiO}_2$ ,  $\text{B}_2\text{O}_3$ ,  $\text{Al}_2\text{O}_3$ ,  $\text{SnO}_2$ , BaO, NiO,  $\text{MoO}_3$ ,  $\text{Ta}_2\text{O}_5$ ,  $\text{Fe}_2\text{O}_3$  and  $\text{Cr}_2\text{O}_3$ . It will be evident from the following description that the composition of the sintered body is different from that of an oxide varistor according to this invention. According to this patent the content of  $\text{SnO}_2$  or  $\text{TiO}_2$  is as low as 0.05 to 10 mol % and it is impossible to attain a predetermined performance in the practice of this invention. Furthermore, the resistor represents a relatively great change when electric current is supplied for a load life test.

An object of this invention is to provide an oxide varistor having a greater voltage nonlinear coefficient ( $\alpha > 30$ ).

Another object of this invention is to provide a high performance oxide varistor capable of representing a lower rising voltage, a small change with temperature, a high surge resistance and a smaller change with time.

The other object will be apparent from the following description.

In accordance with this invention there is provided an oxide varistor prepared from a basic composition formed of 70 to 14 mol % of at least one  $\text{Me}'\text{O}_2$ , 29 to 85 mol % of ZnO and 1 to 20 mol % of  $\text{Sb}_2\text{O}_3$ , 1 to 20 % by weight of  $\text{Bi}_2\text{O}_3$ , and 0.5 to 10 % by weight of at least one  $\text{Me}''\text{O}_2$  based on said basic composition, wherein said  $\text{Me}'$  is a metal selected from the group consisting of Ti, Sn and Zr, and said  $\text{Me}''$  is a metal selected from the group consisting of Fe, Cr, Mn and Co.

This invention can be more fully understood from the following detailed description when taken in connection with reference to the accompanying drawings, in which:

FIG. 1 shows the content of  $\text{Sb}_2\text{O}_3$  and the resistivity of an  $\text{Me}'\text{O}_2\text{-ZnO-Sb}_2\text{O}_3$  system in which the molar ratio of  $\text{Me}'\text{O}$  to ZnO is rendered constant;

FIG. 2 shows the molar ratio of  $\text{Me}'\text{O}_2$  to ZnO and the resistivity of the  $\text{Me}'\text{O}_2\text{-ZnO-Sb}_2\text{O}_3$  system in which the content of  $\text{Sb}_2\text{O}_3$  is rendered constant; and

FIGS. 3A to 6C show a relation between the content of  $\text{Bi}_2\text{O}_3$  and the voltage nonlinear coefficient  $\alpha$  of an  $\text{Me}'\text{O}_2\text{-ZnO-Sb}_2\text{O}_3\text{-Bi}_2\text{O}_3\text{-Me}''\text{O}_2$  system in which  $\text{Me}''\text{O}_2$  is used as a parameter.

An oxide varistor according to this invention can be prepared in the following manners. Accurately weighed out raw material metal oxides having a predetermined composition ratio are mixed together at a ball mill, etc., and after preliminarily sintered at a relatively low temperature, for example, at 600° to 900°C, are powdered by the ball mill. As raw material used in this case, use

may be made of metal compound, such as hydroxide, carbonate, oxalate, etc., which is convertible into oxide upon heating. The powder so obtained is mixed with a binder such as polyvinyl alcohol, etc. The mixture is shaped, under pressure of about 100 to 1,000 Kg/cm<sup>2</sup>, into a disc having a diameter of about 20 mm and a thickness of about 1 mm. The disc is sintered generally in an air atmosphere at a temperature of about 1,000° to 1,300°C. During the sintering it is kept at a maximum temperature for about 1 to 6 hours. Then, electrodes are baked to the resultant disc to obtain a varistor.

As mentioned above, oxide varistor according to this invention includes a basic composition formed of 70 to 14 mol % of metal dioxide  $Me^I O_2$ , 29 to 85 mol % of ZnO and 1 to 20 mol % of  $Sb_2 O_3$ . The metal dioxide is selected from  $TiO_2$ ,  $SnO_2$ ,  $ZrO_2$  or a mixture thereof.

The content of  $Sb_2 O_3$  is 1 to 20 mol %. When the content (mol %) of  $Sb_2 O_3$  of the basic composition i.e.  $Me^I O_2$ -ZnO- $Sb_2 O_3$  system is varied with the molar ratio of  $Me^I O_2$  to ZnO fixed at 1:2, resistivity values as shown in FIG. 1 are obtained. As will be understood from this figure, when  $Sb_2 O_3$  exceeds 1 mol % the resistivity value is sufficiently lowered and is suitable for use as a varistor. However, when  $Sb_2 O_3$  exceeds 20 mol %, then the resistivity value is increased and is unsuitable for use as a varistor. Even if the resistivity presents no problem, sintered bodies are so porous that no desirable varistor is obtained from the practical viewpoint. It is preferred that the content of  $Sb_2 O_3$  be 5 to 15 mol %.

The contents of  $Me^I O_2$  and ZnO are 70 to 14 mol % and 29 to 85 mol %, respectively. When the molar ratio of  $Me^I O_2$  to ZnO of the base  $Me^I O_2$ -ZnO- $Sb_2 O_3$  is varied with the content of  $Sb_2 O_3$  fixed at 6 mol %, then the resistivity of the basic composition is as shown in FIG. 2. As will be appreciated from this figure, when the content of  $Me^I O_2$  is outside the scope of 70 to 14 mol % and the content of ZnO is outside the scope of 29 to 85 mol %, a resistivity is increased and the composition is unsuitable for the practice of this invention. Even if  $Me^I$  is replaced by Ti, Sn or Zr, the same trend will also be observed. Where it is desired to obtain a varistor having a relatively great voltage nonlinear coefficient, it is preferred that the content of  $Me^I O_2$  be in the range of 60 to 30 mol % and the content of ZnO be in the range of 35 to 57 mol %. When it is desired to obtain a varistor whose rising voltage is relatively low, it is preferred that the content of  $Me^I O_2$  be 14 to 20 mol % or around 70 mol % and the content of ZnO be 66 to 85 mol % or around 30 mol %.

An oxide varistor according to this invention contains, as an additive to the base  $Me^I O_2$ -ZnO- $Sb_2 O_3$  composition, 1 to 20 weight % of  $Bi_2 O_3$  and 0.5 to 10 weight % of  $Me^{II} O_3$ . The  $Me^{II} O_3$  is selected from  $Fe_2 O_3$ ,  $Cr_2 O_3$ ,  $Mn_2 O_3$ ,  $Co_2 O_3$  or a mixture thereof. Determination was made of the voltage nonlinear coefficient  $\alpha$  of resistors obtained by adding varying amounts of  $Bi_2 O_3$  to a basic composition formed of 30 mol % of  $Me^I O_2$ , 60 mol % of ZnO and 10 mol % of  $Sb_2 O_3$  in which  $Me^{II} O_3$  is used as a parameter. The results are shown in FIGS. 3A to 6C. Figures with the suffix *a* added show the case where  $Me^I$  is Ti; figures with the suffix *b* added show the case where  $Me^I$  is Sn; and figures with the suffix *c* added show the case where  $Me^I$

is Zr. FIGS. 3A to 3C show the case where  $Me^{II}$  is Fe; FIGS. 4A to 4C where  $Me^{II}$  is Cr; FIGS. 5A to 5C where  $Me^{II}$  is Mn; and FIGS. 6A to 6C where  $Me^{II}$  is Co.

As will be understood from FIGS. 3A to 6C, when the contents of  $Bi_2 O_3$  and  $Me^{II} O_3$  are outside the scope indicated, a varistor whose voltage nonlinear coefficient is great ( $\alpha > 30$ ) is not obtained. Furthermore, those outside the scope have the drawback that a high rise voltage is involved. Even when a composition is outside the scope, there may be obtained a varistor whose voltage nonlinear coefficient exceeds 30. However, the varistor is higher (about 1.5 to 2 times higher) in its rise voltage than a varistor according to this invention which shows a voltage nonlinear coefficient of much the same magnitude. Therefore, it is difficult to handle as well as to be put to practical use.

The above-mentioned voltage-current characteristics are not varied in any composition of this invention even when Ag or an In-Ga alloy is used as electrode material.

An oxide varistor according to this invention has as high a voltage nonlinear coefficient  $\alpha$  as more than 30 and presents extremely small changes with temperature in the rising voltage and a high surge resistance, thus attaining a high performance. Therefore, the varistor is suitably applicable to an arrester, a surge suppressor for vacuum breaker, etc., as well as to the protection of communication instruments against surge and the suppression of abnormal voltage involved in a microwave oven.

Furthermore, an oxide varistor according to this invention can be manufactured at lower cost, since the raw material is obtained at low cost.

This invention will be more fully understood upon reading the following examples.

## EXAMPLES

Mixtures were prepared as shown in tables by adding to a basic composition formed of 75 to 9 mol % of  $Me^I O_2$ , 24 to 90 mol % of ZnO and 1 to 22 mol % of  $Sb_2 O_3$  (totalling 100 mol %), 0.5 to 25 wt % of  $Bi_2 O_3$  and 0.3 to 12 wt % of  $Me^{II} O_3$  based on the basic composition, and intimately mixed at a ball mill. The mixtures were preliminarily sintered at 800°C for 1 hour and powdered at a ball mill. Then, the powders were mixed with polyvinyl alcohol acting as a binder and shaped under a pressure of 1,000 Kg/cm<sup>2</sup>. The shaped powders were heated to a temperature ranging 1,100° to 1,300°C and kept at that temperature for 2 hours for sintering, thereby obtaining 147 discs having a diameter of 20 mm and a thickness of 1 mm. Then, silver electrodes were baked to the disc, resulting in a varistor. An elemental Ag or  $Ag_2 O$  may likewise be used as a starting material for silver electrodes. Since the sintered mass is stable to temperature, the electrode could be baked to the sintered disc over a wider range of about 400° to 800°C. Then, determination was made of the voltage-current characteristics of the samples, i.e., a varistor voltage  $V_c$  at room temperature and a voltage nonlinear coefficient  $\alpha$  using a standard method. The results are shown in Tables I to III. Table I shows the case where  $Me^I$  is Ti; Table II where  $Me^I$  is Sn; and Table III where  $Me^I$  is Zr.

Table I

| Sample No | Main component<br>(mol %) |     |                                |                                | Supplemental<br>component (wt %) | Vc<br>(V) | $\alpha$ |       |       |
|-----------|---------------------------|-----|--------------------------------|--------------------------------|----------------------------------|-----------|----------|-------|-------|
|           | TiO <sub>2</sub>          | ZnO | Sb <sub>2</sub> O <sub>3</sub> | Bi <sub>2</sub> O <sub>3</sub> |                                  |           |          |       |       |
| Control   | 1                         | 70  | 29                             | 1                              | 1                                |           | 306      | 11.0  |       |
|           | 2                         | "   | "                              | "                              | Me=Fe                            | 0.6       | 143      | 34.1  |       |
|           | 3                         | "   | "                              | "                              | Me=Cr                            | "         | 131      | 32.8  |       |
|           | 4                         | "   | "                              | "                              | Me=Mn                            | "         | 138      | 33.6  |       |
|           | 5                         | "   | "                              | "                              | Me=Co                            | "         | 148      | 34.7  |       |
|           | 6                         | 60  | 35                             | 5                              | 5                                |           | 557      | 25.4  |       |
| Control   | 7                         | "   | "                              | "                              | Me=Fe                            | 2.0       | 286      | 73.2  |       |
|           | 8                         | "   | "                              | "                              | Me=Cr                            | "         | 274      | 72.1  |       |
|           | 9                         | "   | "                              | "                              | Me=Mn                            | "         | 280      | 72.5  |       |
|           | 10                        | "   | "                              | "                              | Me=Co                            | "         | 293      | 74.0  |       |
|           | 11                        | "   | "                              | "                              | Me=Fe                            | 1.0       | 295      | 74.6  |       |
|           | 12                        | "   | "                              | "                              | Me=Cr                            | "         |          |       |       |
| Control   | 13                        | 50  | 42                             | 8                              | 7                                | Me=Mn     | "        | 297   | 74.8  |
|           | 14                        | "   | "                              | "                              | Me=Co                            | "         |          |       |       |
|           | 15                        | "   | "                              | "                              | Me=Fe                            | 4.0       | 726      | 41.4  |       |
|           | 16                        | "   | "                              | "                              | Me=Cr                            | "         | 425      | 97.5  |       |
|           | 17                        | "   | "                              | "                              | Me=Mn                            | "         | 414      | 96.3  |       |
|           | 18                        | "   | "                              | "                              | Me=Co                            | "         | 420      | 96.9  |       |
| Control   | 19                        | 40  | 50                             | 10                             | 9.5                              | Me=Fe     | 1.0      | 433   | 98.6  |
|           | 20                        | "   | "                              | "                              | Me=Cr                            | "         | 438      | 99.0  |       |
|           | 21                        | "   | "                              | "                              | Me=Mn                            | "         |          |       |       |
|           | 22                        | "   | "                              | "                              | Me=Co                            | "         |          |       |       |
|           | 23                        | "   | "                              | "                              | Me=Fe                            | 1.6       | 776      | 45.8  |       |
|           | 24                        | "   | "                              | "                              | Me=Cr                            | "         | 461      | 111.3 |       |
| Control   | 25                        | "   | "                              | "                              | Me=Mn                            | "         | 452      | 110.0 |       |
|           | 26                        | 30  | 57                             | 13                             | 12                               | Me=Co     | "        | 458   | 111.1 |
|           | 27                        | "   | "                              | "                              | Me=Fe                            | 6.0       | 474      | 115.4 |       |
|           | 28                        | "   | "                              | "                              | Me=Cr                            | "         | 479      | 116.2 |       |
|           | 29                        | "   | "                              | "                              | Me=Mn                            | "         |          |       |       |
|           | 30                        | "   | "                              | "                              | Me=Co                            | "         |          |       |       |
| Control   | 31                        | 20  | 64                             | 16                             | 14                               | Me=Fe     | 8.0      | 542   | 24.4  |
|           | 32                        | "   | "                              | "                              | Me=Cr                            | "         | 273      | 60.1  |       |
|           | 33                        | "   | "                              | "                              | Me=Mn                            | "         | 260      | 58.8  |       |
|           | 34                        | "   | "                              | "                              | Me=Co                            | "         | 267      | 58.2  |       |
|           | 35                        | "   | "                              | "                              | Me=Fe                            | 2.0       | 282      | 61.3  |       |
|           | 36                        | "   | "                              | "                              | Me=Cr                            | "         | 284      | 61.6  |       |
| Control   | 37                        | 14  | 66                             | 20                             | 20                               | Me=Mn     | "        |       |       |
|           | 38                        | "   | "                              | "                              | Me=Co                            | "         |          |       |       |
|           | 39                        | "   | "                              | "                              | Me=Fe                            | 10.0      | 315      | 11.5  |       |
|           | 40                        | "   | "                              | "                              | Me=Cr                            | "         | 163      | 36.0  |       |
|           | 41                        | "   | "                              | "                              | Me=Mn                            | "         | 151      | 35.2  |       |
|           | 42                        | 14  | 85                             | 1                              | 20                               | Me=Co     | "        | 148   | 34.6  |
| Control   | 43                        | "   | "                              | "                              | Me=Fe                            | 0.5       | 170      | 37.3  |       |
|           | 44                        | "   | "                              | "                              | Me=Cr                            | "         | 291      | 10.8  |       |
|           | 45                        | "   | "                              | "                              | Me=Mn                            | "         | 125      | 32.7  |       |
|           | 46                        | "   | "                              | "                              | Me=Co                            | "         | 117      | 31.9  |       |
|           | 47                        | "   | "                              | "                              | Me=Fe                            | "         | 120      | 32.2  |       |
|           | 48                        | 75  | 24                             | 1                              | 25                               | Me=Cr     | "        | 132   | 33.6  |
| Control   | 49                        | 9   | 90                             | 1                              | 0.5                              | Me=Mn     | "        | 293   | 16.9  |
|           | 49                        | 48  | 30                             | 22                             | 6                                | Me=Co     | 4.0      | 258   | 14.0  |
|           |                           |     |                                |                                |                                  | Me=Mn     | "        | 327   | 21.1  |

Table II

| Sample No. | Main Component<br>(mol %) |     |                                |                                | Supplemental<br>component (wt %) | Vc<br>(V) | $\alpha$ |      |      |
|------------|---------------------------|-----|--------------------------------|--------------------------------|----------------------------------|-----------|----------|------|------|
|            | SnO <sub>2</sub>          | ZnO | Sb <sub>2</sub> O <sub>3</sub> | Bi <sub>2</sub> O <sub>3</sub> |                                  |           |          |      |      |
| Control    | 50                        | 70  | 29                             | 1                              | 1                                |           | 309      | 11.2 |      |
|            | 51                        | "   | "                              | "                              | Me=Fe                            | 0.6       | 130      | 31.5 |      |
|            | 52                        | "   | "                              | "                              | Me=Cr                            | "         | 136      | 32.4 |      |
|            | 53                        | "   | "                              | "                              | Me=Mn                            | "         | 142      | 33.1 |      |
|            | 54                        | "   | "                              | "                              | Me=Co                            | "         | 147      | 33.8 |      |
|            | 55                        | 60  | 35                             | 5                              | 5                                |           | 568      | 25.9 |      |
| Control    | 56                        | "   | "                              | "                              | Me=Fe                            | 2.0       | 281      | 72.5 |      |
|            | 57                        | "   | "                              | "                              | Me=Cr                            | "         | 286      | 73.0 |      |
|            | 58                        | "   | "                              | "                              | Me=Mn                            | "         | 295      | 74.2 |      |
|            | 59                        | "   | "                              | "                              | Me=Co                            | "         | 299      | 75.3 |      |
|            | 60                        | "   | "                              | "                              | Me=Fe                            | 1.0       | 302      | 75.6 |      |
|            | 61                        | "   | "                              | "                              | Me=Cr                            | "         |          |      |      |
| Control    | 62                        | 50  | 42                             | 8                              | 7                                | Me=Mn     | "        | 304  | 75.8 |
|            | 63                        | "   | "                              | "                              | Me=Co                            | "         |          |      |      |
|            | 64                        | "   | "                              | "                              | Me=Fe                            | 4.0       | 735      | 42.5 |      |
|            | "                         | "   | "                              | "                              | Me=Cr                            | "         | 407      | 95.2 |      |

Table II -Continued

| Sample No. | Main Component (mol %) |     |                                |                                | Supplemental component (wt %)   |      | Vc (V) | $\alpha$ |
|------------|------------------------|-----|--------------------------------|--------------------------------|---------------------------------|------|--------|----------|
|            | SnO <sub>2</sub>       | ZnO | Sb <sub>2</sub> O <sub>3</sub> | Bi <sub>2</sub> O <sub>3</sub> | Me <sup>II</sup> O <sub>3</sub> |      |        |          |
| 65         | "                      | "   | "                              | "                              | Me=Mn                           | "    | 420    | 96.3     |
| 66         | "                      | "   | "                              | "                              | Me=Co                           | "    | 426    | 97.7     |
| 67         | "                      | "   | "                              | "                              | Me=Fe                           | 1.0  | 431    | 98.4     |
|            |                        |     |                                |                                | Me=Cr                           | "    |        |          |
|            |                        |     |                                |                                | Me=Mn                           | "    |        |          |
|            |                        |     |                                |                                | Me=Co                           | "    |        |          |
| Control 68 | 40                     | 50  | 10                             | 9.5                            |                                 |      | 783    | 47.2     |
| 69         | "                      | "   | "                              | "                              | Me=Fe                           | 4.8  | 446    | 107.5    |
| 70         | "                      | "   | "                              | "                              | Me=Cr                           | "    | 451    | 109.0    |
| 71         | "                      | "   | "                              | "                              | Me=Mn                           | "    | 457    | 110.8    |
| 72         | "                      | "   | "                              | "                              | Me=Co                           | "    | 464    | 112.3    |
| 73         | "                      | "   | "                              | "                              | Me=Fe                           | 1.6  | 466    | 113.1    |
|            |                        |     |                                |                                | Me=Cr                           | "    |        |          |
|            |                        |     |                                |                                | Me=Mn                           | "    |        |          |
| 74         | "                      | "   | "                              | "                              | Me=Cr                           | "    | 472    | 113.9    |
|            |                        |     |                                |                                | Me=Mn                           | "    |        |          |
|            |                        |     |                                |                                | Me=Co                           | "    |        |          |
| Control 75 | 30                     | 57  | 13                             | 12                             |                                 |      | 663    | 36.6     |
| 76         | "                      | "   | "                              | "                              | Me=Fe                           | 6.0  | 355    | 78.8     |
| 77         | "                      | "   | "                              | "                              | Me=Cr                           | "    | 360    | 79.5     |
| 78         | "                      | "   | "                              | "                              | Me=Mn                           | "    | 367    | 81.1     |
| 79         | "                      | "   | "                              | "                              | Me=Co                           | "    | 371    | 82.4     |
| Control 80 | 20                     | 64  | 16                             | 14                             |                                 |      | 525    | 24.0     |
| 81         | "                      | "   | "                              | "                              | Me=Fe                           | 8.0  | 250    | 55.9     |
| 82         | "                      | "   | "                              | "                              | Me=Cr                           | "    | 256    | 57.2     |
| 83         | "                      | "   | "                              | "                              | Me=Mn                           | "    | 263    | 58.3     |
| 84         | "                      | "   | "                              | "                              | Me=Co                           | "    | 272    | 59.4     |
| 85         | "                      | "   | "                              | "                              | Me=Fe                           | 2.0  | 277    | 60.1     |
|            |                        |     |                                |                                | Me=Cr                           | "    |        |          |
|            |                        |     |                                |                                | Me=Mn                           | "    |        |          |
|            |                        |     |                                |                                | Me=Co                           | "    |        |          |
| Control 86 | 14                     | 66  | 20                             | 20                             |                                 |      | 318    | 11.8     |
| 87         | "                      | "   | "                              | "                              | Me=Fe                           | 10.0 | 153    | 34.6     |
| 88         | "                      | "   | "                              | "                              | Me=Cr                           | "    | 165    | 35.0     |
| 89         | "                      | "   | "                              | "                              | Me=Mn                           | "    | 174    | 35.9     |
| 90         | "                      | "   | "                              | "                              | Me=Co                           | "    | 181    | 36.7     |
| Control 91 | 14                     | 85  | 1                              | 20                             |                                 |      | 288    | 10.6     |
| 92         | "                      | "   | "                              | "                              | Me=Fe                           | 0.5  | 116    | 31.1     |
| 93         | "                      | "   | "                              | "                              | Me=Cr                           | "    | 120    | 32.4     |
| 94         | "                      | "   | "                              | "                              | Me=Mn                           | "    | 127    | 32.9     |
| 95         | "                      | "   | "                              | "                              | Me=Co                           | "    | 133    | 33.5     |
| Control 96 | 75                     | 24  | 1                              | 25                             | Me=Fe                           | 0.3  | 297    | 17.8     |
| Control 97 | 9                      | 90  | 1                              | 0.5                            | Me=Cr                           | 12.0 | 255    | 13.7     |
| Control 98 | 48                     | 30  | 22                             | 6                              | Me=Mn                           | 4.0  | 320    | 20.4     |

Table III

| Sample No.  | Main component (mol %) |     |                                |                                | Supplemental component (wt %)   |     | Vc (V) | $\alpha$ |
|-------------|------------------------|-----|--------------------------------|--------------------------------|---------------------------------|-----|--------|----------|
|             | ZrO <sub>2</sub>       | ZnO | Sb <sub>2</sub> O <sub>3</sub> | Bi <sub>2</sub> O <sub>3</sub> | Me <sup>II</sup> O <sub>3</sub> |     |        |          |
| Control 99  | 70                     | 29  | 1                              | 1                              |                                 |     | 303    | 10.9     |
| 100         | "                      | "   | "                              | "                              | Me=Fe                           | 0.6 | 154    | 35.1     |
| 101         | "                      | "   | "                              | "                              | Me=Cr                           | "   | 138    | 33.0     |
| 102         | "                      | "   | "                              | "                              | Me=Mn                           | "   | 142    | 34.3     |
| 103         | "                      | "   | "                              | "                              | Me=Co                           | "   | 160    | 36.2     |
| Control 104 | 60                     | 35  | 5                              | 5                              |                                 |     | 549    | 26.5     |
| 105         | "                      | "   | "                              | "                              | Me=Fe                           | 2.0 | 290    | 74.4     |
| 106         | "                      | "   | "                              | "                              | Me=Cr                           | "   | 273    | 73.0     |
| 107         | "                      | "   | "                              | "                              | Me=Mn                           | "   | 284    | 73.6     |
| 108         | "                      | "   | "                              | "                              | Me=Co                           | "   | 295    | 75.2     |
| 109         | "                      | "   | "                              | "                              | Me=Fe                           | 1.0 | 297    | 75.8     |
|             |                        |     |                                |                                | Me=Cr                           | "   |        |          |
|             |                        |     |                                |                                | Me=Mn                           | "   |        |          |
| 110         | "                      | "   | "                              | "                              | Me=Co                           | "   | 301    | 76.1     |
| Control 111 | 50                     | 42  | 8                              | 7                              |                                 |     | 724    | 40.9     |
| 112         | "                      | "   | "                              | "                              | Me=Fe                           | 4.0 | 436    | 98.7     |
| 113         | "                      | "   | "                              | "                              | Me=Cr                           | "   | 425    | 98.0     |
| 114         | "                      | "   | "                              | "                              | Me=Mn                           | "   | 418    | 97.1     |
| 115         | "                      | "   | "                              | "                              | Me=Co                           | "   | 445    | 99.6     |
| 116         | "                      | "   | "                              | "                              | Me=Fe                           | 1.0 | 451    | 100.3    |
|             |                        |     |                                |                                | Me=Cr                           | "   |        |          |
|             |                        |     |                                |                                | Me=Mn                           | "   |        |          |
|             |                        |     |                                |                                | Me=Co                           | "   |        |          |
| Control 117 | 40                     | 50  | 10                             | 9.5                            |                                 |     | 757    | 46.2     |
| 118         | "                      | "   | "                              | "                              | Me=Fe                           | 4.8 | 473    | 114.6    |
| 119         | "                      | "   | "                              | "                              | Me=Cr                           | "   | 465    | 112.3    |
| 120         | "                      | "   | "                              | "                              | Me=Mn                           | "   | 461    | 111.5    |
| 121         | "                      | "   | "                              | "                              | Me=Co                           | "   | 480    | 115.8    |
| 122         | "                      | "   | "                              | "                              | Me=Fe                           | 1.6 | 484    | 116.1    |
|             |                        |     |                                |                                | Me=Cr                           | "   |        |          |
|             |                        |     |                                |                                | Me=Mn                           | "   |        |          |
| 123         | 40                     | 50  | 10                             | 9.5                            | Me=Cr                           | 1.6 | 486    | 116.3    |
|             |                        |     |                                |                                | Me=Mn                           | "   |        |          |
|             |                        |     |                                |                                | Me=Co                           | "   |        |          |

Table III - Continued

| Sample No.  | Main component<br>(mol %) |     |                                |                                | Supplemental<br>component (wt %) | Vc<br>(V) | $\alpha$ |
|-------------|---------------------------|-----|--------------------------------|--------------------------------|----------------------------------|-----------|----------|
|             | ZrO <sub>2</sub>          | ZnO | Sb <sub>2</sub> O <sub>3</sub> | Bi <sub>2</sub> O <sub>3</sub> |                                  |           |          |
| Control 124 | 30                        | 57  | 13                             | 12                             |                                  | 657       | 35.8     |
| 125         | "                         | "   | "                              | "                              | Me=Fe                            | 361       | 79.6     |
| 126         | "                         | "   | "                              | "                              | Me=Cr                            | 350       | 77.7     |
| 127         | "                         | "   | "                              | "                              | Me=Mn                            | 344       | 76.7     |
| 128         | "                         | "   | "                              | "                              | Me=Co                            | 365       | 80.2     |
| Control 129 | 20                        | 64  | 16                             | 14                             |                                  | 545       | 25.0     |
| 130         | "                         | "   | "                              | "                              | Me=Fe                            | 282       | 61.5     |
| 131         | "                         | "   | "                              | "                              | Me=Cr                            | 271       | 60.3     |
| 132         | "                         | "   | "                              | "                              | Me=Mn                            | 264       | 59.8     |
| 133         | "                         | "   | "                              | "                              | Me=Co                            | 287       | 62.4     |
| 134         | "                         | "   | "                              | "                              | Me=Fe                            | 290       | 62.7     |
|             |                           |     |                                |                                | Me=Cr                            |           |          |
|             |                           |     |                                |                                | Me=Mn                            |           |          |
|             |                           |     |                                |                                | Me=Co                            |           |          |
| Control 135 | 14                        | 66  | 20                             | 20                             |                                  | 309       | 11.1     |
| 136         | "                         | "   | "                              | "                              | Me=Fe                            | 173       | 38.0     |
| 137         | "                         | "   | "                              | "                              | Me=Cr                            | 161       | 36.9     |
| 138         | "                         | "   | "                              | "                              | Me=Mn                            | 155       | 36.2     |
| 139         | "                         | "   | "                              | Me=Co                          | "                                | 182       | 39.3     |
| Control 140 | 14                        | 85  | 1                              | 20                             |                                  | 290       | 10.5     |
| 141         | "                         | "   | "                              | "                              | Me=Fe                            | 0.5       | 130      |
| 142         | "                         | "   | "                              | "                              | Me=Cr                            | "         | 122      |
| 143         | "                         | "   | "                              | "                              | Me=Mn                            | "         | 118      |
| 144         | "                         | "   | "                              | "                              | Me=Co                            | "         | 137      |
| Control 145 | 75                        | 24  | 1                              | 25                             | Me=Fe                            | 0.3       | 291      |
| Control 146 | 9                         | 90  | 1                              | 0.5                            | Me=Cr                            | 12.0      | 256      |
| Control 147 | 48                        | 30  | 22                             | 6                              | Me=Mn                            | 4.0       | 320      |
|             |                           |     |                                |                                |                                  |           | 20.3     |

As will be appreciated from Tables I to III, the varistor having a basic composition formed of 60 to 30 mol % of Me'<sub>2</sub>O<sub>3</sub>, 35 to 57 mol % of ZnO and 5 to 15 mol % of Sb<sub>2</sub>O<sub>3</sub>, exhibits an extremely high voltage nonlinear coefficient. Furthermore, the varistor having a basic composition formed of 14 to 20 mol % or about 70 mol % of Me'<sub>2</sub>O<sub>3</sub>, 64 to 85 mol % or about 30 mol % of ZnO and 1 to 20 mol % of Sb<sub>2</sub>O<sub>3</sub> has a particularly low rise voltage.

With respect to some of the above-mentioned examples determination was made of the change with temperature in the rising voltage (Vc) and surge resistance involved in a pulse current of 8  $\times$  20  $\mu$ s. The results are shown in Table IV in which the voltage nonlinear coefficient  $\alpha$  as shown in Tables I to III is restated.

Table IV

| Sample No. | Change with<br>temperature<br>in the rising<br>voltage (%/°C) | Surge<br>resistance<br>(A/cm <sup>2</sup> ) | Voltage<br>nonlinear<br>coefficient<br>$\alpha$ |
|------------|---------------------------------------------------------------|---------------------------------------------|-------------------------------------------------|
| Control 1  | -0.004                                                        | 2570                                        | 11.0                                            |
| " 13       | -0.005                                                        | 2760                                        | 41.4                                            |
| " 26       | -0.005                                                        | 2830                                        | 36.2                                            |
| " 48       | -0.008                                                        | 2180                                        | 14.0                                            |
| " 50       | -0.005                                                        | 2550                                        | 11.2                                            |
| " 62       | -0.004                                                        | 2840                                        | 42.5                                            |
| " 75       | -0.004                                                        | 2730                                        | 36.6                                            |
| " 97       | -0.009                                                        | 2220                                        | 13.7                                            |
| " 99       | -0.005                                                        | 2540                                        | 10.9                                            |
| " 111      | -0.005                                                        | 2710                                        | 40.9                                            |
| " 129      | -0.004                                                        | 2820                                        | 25.0                                            |
| " 146      | -0.008                                                        | 2130                                        | 13.7                                            |
| 3          | -0.003                                                        | 3390                                        | 32.8                                            |
| 5          | -0.002                                                        | 3620                                        | 34.7                                            |
| 9          | -0.002                                                        | 3970                                        | 72.5                                            |
| 16         | -0.003                                                        | 4220                                        | 96.9                                            |
| 21         | -0.001                                                        | 4630                                        | 110.0                                           |
| 24         | -0.002                                                        | 4950                                        | 116.2                                           |
| 28         | -0.001                                                        | 4110                                        | 78.1                                            |
| 34         | -0.003                                                        | 3870                                        | 58.2                                            |
| 38         | -0.002                                                        | 3640                                        | 36.0                                            |
| 43         | -0.001                                                        | 3380                                        | 32.7                                            |
| 53         | -0.002                                                        | 3360                                        | 33.1                                            |
| 56         | -0.003                                                        | 3580                                        | 72.5                                            |
| 59         | -0.001                                                        | 3930                                        | 75.3                                            |
| 66         | -0.002                                                        | 4240                                        | 97.8                                            |
| 71         | -0.002                                                        | 4610                                        | 110.8                                           |
| 74         | -0.003                                                        | 4950                                        | 113.9                                           |

Table IV - Continued

| Sample No. | Change with<br>temperature<br>in the rising<br>voltage (%/°C) | Surge<br>resistance<br>(A/cm <sup>2</sup> ) | Voltage<br>nonlinear<br>coefficient<br>$\alpha$ |
|------------|---------------------------------------------------------------|---------------------------------------------|-------------------------------------------------|
| 78         | -0.002                                                        | 4100                                        | 81.1                                            |
| 84         | -0.001                                                        | 3890                                        | 59.4                                            |
| 88         | -0.002                                                        | 3630                                        | 35.0                                            |
| 93         | -0.001                                                        | 3420                                        | 32.4                                            |
| 100        | -0.003                                                        | 3240                                        | 35.1                                            |
| 102        | -0.002                                                        | 3580                                        | 34.3                                            |
| 105        | -0.003                                                        | 3880                                        | 74.4                                            |
| 113        | -0.002                                                        | 4070                                        | 98.0                                            |
| 118        | -0.002                                                        | 4560                                        | 114.6                                           |
| 121        | -0.001                                                        | 4930                                        | 115.8                                           |
| 125        | -0.002                                                        | 4440                                        | 79.6                                            |
| 131        | -0.001                                                        | 3950                                        | 60.3                                            |
| 134        | -0.003                                                        | 3720                                        | 62.7                                            |
| 139        | -0.001                                                        | 3490                                        | 39.3                                            |

As will be understood from Table IV, the change with temperature in the rising voltage of the oxide varistor according to this invention is below -0.003 %/°C and the varistor is very favorably compared with the conventional SiC varistor (-0.1 %/°C) and zener diode (-0.1 %/°C). Furthermore, the surge resistance of the varistor according to this invention is more than 3,000 A/cm<sup>2</sup> and very favorably compared with the conventional zinc oxide varistor element (2,000 A/cm<sup>2</sup>) and zener diode (20 A/cm<sup>2</sup>).

With the varistors outside the scope of this invention, for example, the sample Nos. 13, 26, 62, 75, 111, etc., the voltage nonlinear coefficient  $\alpha$  exceeds 30 and they are favorably compared with some of the varistors according to this invention. However, they are inferior, in the change with temperature in the rising voltage as well as in the surge resistance, to the varistors according to this invention.

The varistor according to this invention was supplied with an electric power of 1 watt for a load life test and kept at 70°C for 500 hours. Therefore, the variation of the voltage nonlinear coefficient  $\alpha$  was determined. The results are shown below in comparison with the re-

65

sitors of U.S. Pat. No. 3,663,458 which are described in Table 12 of this patent.

Table V

| Sample No.                     | Variation of voltage nonlinear coefficient $\alpha$ after load life test (%) |
|--------------------------------|------------------------------------------------------------------------------|
| 18                             | -0.8                                                                         |
| 35                             | -0.9                                                                         |
| 72                             | -0.3                                                                         |
| 87                             | -0.7                                                                         |
| 110                            | -0.6                                                                         |
| 133                            | -0.8                                                                         |
| 139                            | -0.2                                                                         |
| Control                        |                                                                              |
| ZnO                            | 99.5                                                                         |
| Sb <sub>2</sub> O <sub>3</sub> | 0.5                                                                          |
| ZnO                            | 99.5                                                                         |
| SnO <sub>2</sub>               | 0.5                                                                          |

From this table it will be understood that the varistor according to this invention undergoes a very small change with time. Though Me' is used in a single compound, the same result is obtained even when it is used in a mixed form.

What we claim is:

1. An oxide varistor prepared from a basic composition consisting of a total of 70 to 14 mol % of at least one compound of the formula Me'O<sub>2</sub>, 29 to 85 mol % of ZnO and 1 to 20 mol % of Sb<sub>2</sub>O<sub>3</sub>, and containing 1 to 20 % by weight of Bi<sub>2</sub>O<sub>3</sub>, and a total of 0.5 to 10 % by weight of at least one Me''O<sub>3</sub> based on the weight

of said basic composition, wherein said Me' is selected from the group consisting of Ti, Sn and Zr, said Me'' is selected from the group consisting of Fe, Cr, Mn and Co.

5. 2. The oxide varistor according to claim 1 wherein said basic composition consists of 60 to 30 mol % of Me'O<sub>2</sub>, 35 to 57 mol % of ZnO and 5 to 15 mol % of Sb<sub>2</sub>O<sub>3</sub>.

10 3. The oxide varistor according to claim 1, wherein the amount of said Me'O<sub>2</sub> of the basic composition is 20 to 14 mol % and the amount of said ZnO of the basic composition is 66 to 85 mol %.

15 4. The oxide varistor according to claim 1, wherein the amount of said Me'O<sub>2</sub> of the basic composition is about 70 mol % and the amount of said ZnO of the basic composition is about 30 mol %.

20 5. An oxide varistor having a nonlinear voltage coefficient ( $\alpha$ ) greater than 30, a change with temperature in rising voltage of less than -0.003%/°C and a surge resistance of more than 3,000 A/cm<sup>2</sup>, said oxide varistor being prepared from a basic composition consisting of a total of 70 to 14 mol % of at least one compound of the formula Me'O<sub>2</sub>, 29 to 85 mol % of ZnO and 1 to 20 mol % of Sb<sub>2</sub>O<sub>3</sub>, and containing 1 to 20 % by weight of Bi<sub>2</sub>O<sub>3</sub>, and a total of 0.5 to 10 % by weight of at least one Me''O<sub>3</sub> based on the weight of said basic composition, wherein said Me' is selected from the group consisting of Ti, Sn and Zr, and said Me'' is selected from the group consisting of Fe, Cr, Mn and Co.

\* \* \* \* \*

35

40

45

50

55

60

65